

## UNITED STATES PATENT OFFICE

2,326,102

## DIESEL FUEL

Edwin M. Nygaard and John H. McCracken,  
Woodbury, and Francis M. Seger, Pitman, N. J.,  
assignors to Socony-Vacuum Oil Company, In-  
corporated, New York, N. Y., a corporation of  
New York

No Drawing. Application April 24, 1941,  
Serial No. 390,102

13 Claims. (Cl. 44—57)

This invention has to do in a general way with fuels for internal combustion engines of the compression ignition or Diesel type and is more particularly concerned with the improvement of such fuels by the addition of characterizing ingredients for the purpose of modifying or controlling the combustion characteristics.

In the operation of Diesel engines, where the fuel is injected into a combustion space, it is important to the attainment of maximum efficiency that the delay period between injection and ignition be short. Improperly delayed ignition in a Diesel engine gives rise to the phenomenon known as "knocking," which is due to improper coordination of combustion and cylinder conditions. By accelerating the ignition of Diesel fuel, it is possible to lower the compression pressure. This insures spontaneous ignition without combustion shock, thereby increasing the ease of starting and the smoothness with which combustion takes place. Also, the low compression pressure permits less weight in the engine and a lower cost per given power output. It is obvious, therefore, that enhanced speed of ignition is a characteristic which is highly desirable in a Diesel fuel.

It has been found that the ignition quality of the fuel oils normally classified as Diesel fuels can be improved by the addition of small amounts of certain compounds which will act as ignition accelerators, thereby decreasing the ignition delay period. This offers a means for improving the better grades of Diesel fuels and a means for widening the range of available fuels by raising the ignition quality of the lower grades to a point where they can be satisfactorily used.

This invention is predicated upon the discovery that Diesel fuels of improved ignition quality can be obtained by admixing with the fuel a minor proportion of the compound or reaction product obtained by reacting perchloromethylmercaptan ( $\text{Cl}_2\text{C.SCl}$ ) with a compound of the general formula  $\text{R}(\text{XH})_n$  or  $\text{R}(\text{XM})_n$ , where  $\text{R}$  represents an alkyl, aryl, alkaryl, or aralkyl radical and  $\text{X}$  is oxygen or sulfur and  $\text{M}$  represents the hydrogen equivalent of a metal and  $n$  is a whole number.

Perchloromethylmercaptan, as indicated by the formula above, is a chlorinated substituted

sulfur chloride and can be prepared by the chlorination of carbon disulfide according to the method of Helfrich and Reid (Jour. Amer. Chem. Soc. 43, 591 (1921)). For example, carbon disulfide containing about .4 per cent by weight of iodine was chlorinated in the absence of direct sunlight at a temperature maintained below 25° C. until the volume of the reaction mixture had doubled. This crude product, which contains carbon tetrachloride and sulfur chloride in addition to perchloromethylmercaptan, is then purified by distillation on a water bath, followed by steam-distillation. The product refined in this way is practically pure.

The secondary reactants represented hereinabove by the general formulae  $\text{R}(\text{XH})_n$  and  $\text{R}(\text{XM})_n$  comprise mono- and poly-hydric alcohols (including mercaptans) and phenols (including thiophenols) and the corresponding metal derivatives, (alcoholates, phenolates, mercaptides, etc.). To facilitate the reaction of the perchloromethylmercaptan and a secondary reactant  $\text{RXH}$ , it is desirable to carry out the reaction in the presence of an alkali metal or its corresponding hydroxide; and when the reaction is carried out in this way, the metal may be present as a substituent replacing the hydrogen in the  $\text{XH}$  group of the secondary reactant and in such an instance, even though the compound used as the secondary reactant has the general formula  $\text{RXH}$ , the compound actually entering into the reaction has the formula  $\text{RXM}$ .

Typical procedures which may be employed in synthesizing the reaction products contemplated herein are illustrated by the following examples:

## EXAMPLE I

## Preparation of reaction product between perchloromethylmercaptan and phenol

One part of phenol was dissolved in 8.6 parts of 2N sodium hydroxide and was treated at intervals with 5-gram portions of perchloromethylmercaptan (40 grams, 1.6 parts in all). The solution was cooled and agitated between each addition. After 15 minutes an oil was extracted with 5.1 parts of ether, the ether extract washed twice with water and dried over anhydrous potassium carbonate. The ether extract was filtered into a distilling flask and the ether re-

moved at room temperature under reduced pressure. The product, amounting to 42 grams, was a pale yellow oil.

EXAMPLE II

*Preparation of reaction product obtained from perchloromethylmercaptan and ethyl alcohol*

To 14.5 parts of absolute ethyl alcohol contained in a 2-liter three-necked flask equipped with a Hershberg wire stirrer and reflux condenser was added 1 part of metallic sodium. The mixture was cooled to control the reaction. When most of the sodium had dissolved, the reaction flask was surrounded with an ice bath and to the cold mixture was slowly added over a period of a half an hour 6.3 parts of perchloromethylmercaptan dissolved in 19.7 parts of petroleum ether. A white precipitate formed immediately. To the product was added 45.5 parts of water, which dissolved the precipitate. The aqueous layer was extracted with an additional 50 cc. (2.3 parts) of petroleum ether. The petroleum ether extracts were combined, washed with water, dried over calcium chloride, and filtered into a distilling flask. The contents of the flask were heated to 50° C. under vacuum to completely remove the petroleum ether. The yield of crude product was 139 grams (6.3 parts).

The examples given above are merely illustrative, and from them the modifications necessary to synthesize reaction products from other compounds within the class typified by the formula RXH will readily appear to those skilled in the art. Other typical compounds which are contemplated for use as the secondary reactant are substituted phenols, such as cresols, trinitro-phenol, xylenols, naphthols, etc., thiophenol and substituted thiophenols, such as thiocresols, thioxyleneols, etc., aliphatic alcohols in general, including monohydric and polyhydric alcohols (glycol, glycerol, etc.), substituted alcohols, such as nitro alcohols, etc., and aliphatic and aralkyl mercaptans in general, including mono-, di-, and tri- mercaptans, benzyl mercaptans, thioglycols, etc., and the metal derivatives (alcoholates, phenolates, and mercaptides) corresponding to the foregoing compounds.

Reaction products have been prepared and tested and found satisfactory as ignition accelerators for Diesel fuels wherein the secondary reactant was selected from the group consisting of phenol, ethyl alcohol, amyl mercaptan, tertiary butyl mercaptan, thiophenol, and benzyl mercaptan. In the class of compounds contemplated herein as secondary reactants, preference is given to phenols, mercaptans and thiophenols. The exact chemical composition of the reaction products contemplated herein is uncertain, but they contain substantial quantities of chlorine and sulfur derived from the perchloromethyl mercaptan,  $\text{Cl}_3\text{CSCl}$ . They are probably predominantly comprised of compounds having the general formulae  $\text{Cl}_3\text{C}-\text{S}-\text{S}-\text{R}$  or  $\text{Cl}_3\text{C}-\text{S}-\text{OR}$ , depending upon whether the secondary reactant is a mercaptan (or mercaptide) or an alcohol (or alcoholate). Because of the uncertainty as to the exact chemical composition of these products, they are defined herein by the method of preparation.

The term Diesel fuel, as used herein, has reference to those non-viscous petroleum fractions commonly denoted in the art as Diesel fuels and to those hydrocarbon products in general whose physical characteristics render them suitable for use in compression ignition engines.

To demonstrate the effectiveness of the reaction products contemplated herein as improving agents for Diesel fuels, blends of typical reaction products were prepared in a straight-run Number 2 fuel oil, and the cetane numbers of the blends were obtained for comparison with the cetane number of the blank fuel oil. The cetane numbers were determined by the proposed method of the A. S. T. M. (A. S. T. M. Proc. 38 I 392 (1938)). The fuel oil used had the following characteristics:

|                                  |       |
|----------------------------------|-------|
| Gravity, °A. P. I.               | 39.8  |
| Flash point (Pensky-Martens °F.) | 172   |
| Aniline point, °F.               | 160.5 |
| 15 A. S. T. M. distillation:     |       |
| Initial °F.                      | 386   |
| 10%                              | 435   |
| 90%                              | 572   |
| End point                        | 614   |
| 20 Diesel index                  | 63.9  |
| Cetane No.                       | 55    |

The cetane number determinations and the extent to which the cetane numbers were improved by the various reaction products are shown in Table I below.

TABLE I

| Substance blended with 55 cetane number fuel                  | Per cent by wt. added | Cetane No. of blend | Increase in cetane No. |
|---------------------------------------------------------------|-----------------------|---------------------|------------------------|
| Reaction product obtained from perchloromethylmercaptan with— |                       |                     |                        |
| Phenol                                                        | 1.0                   | 60.5                | 5.5                    |
| Do                                                            | 1.0                   | 62.0                | 7.0                    |
| 35 Ethyl alcohol                                              | 1.0                   | 58.0                | 3.0                    |
| Amyl mercaptan                                                | 1.0                   | 62.0                | 7.0                    |
| Ethyl                                                         | 1.0                   | 58.0                | 3.0                    |
| Tertiary butyl mercaptan                                      | 1.0                   | 62.0                | 7.0                    |
| Thio-phenol                                                   | 1.0                   | 61.6                | 6.6                    |
| Benzyl mercaptan                                              | 1.0                   | 61.6                | 6.6                    |

40 The reaction products obtained from perchloromethylmercaptan with thio-phenol and benzyl mercaptan were also added to a catalytically cracked Number 2 fuel oil, and the cetane number of the blends were determined. The base fuel has the following characteristics:

|                                  |      |
|----------------------------------|------|
| Gravity, °A. P. I.               | 28.8 |
| Flash point (Pensky-Martens °F.) | 200  |
| Aniline point, °F.               | 122  |

|                              |      |
|------------------------------|------|
| 50 A. S. T. M. distillation: |      |
| Initial °F.                  | 431  |
| 10%                          | 467  |
| 90%                          | 582  |
| End point                    | 629  |
| 55 Diesel index              | 35.1 |
| Cetane number                | 33.0 |

The cetane number determinations are listed in Table II below.

TABLE II

| Substance blended with 33 cetane number fuel                  | Per cent by wt. added | Cetane No. of blend | Increase in cetane No. |
|---------------------------------------------------------------|-----------------------|---------------------|------------------------|
| Reaction product obtained from perchloromethylmercaptan with— |                       |                     |                        |
| Thio-phenol                                                   | 1.0                   | 37.7                | 4.7                    |
| Benzyl mercaptan                                              | 1.0                   | 38.0                | 5.0                    |

70 The reaction products contemplated herein may be used in amounts ranging from about 0.1 per cent to about 5.0 per cent; and it is to be understood that although we have described certain specific procedures and have referred to various specific compounds as the secondary reactants, our invention is not limited thereto but

includes within its scope whatever changes and modifications are fairly encompassed by the appended claims.

**We claim:**

1. An improved Diesel fuel comprising a hydrocarbon fuel oil and in admixture therewith a minor proportion of the oil-miscible product obtained by first reacting perchloromethylmercaptoan with a compound selected from the group consisting of compounds having the general formula  $R(XH)_n$  and  $R(XM)_n$ , wherein R is selected from the group consisting of alkyl, aryl, alkaryl and aralkyl radicals, X is selected from the group consisting of oxygen and sulfur, M is a metal, and n is a whole number, and then separating the oil-miscible reaction product from the unreacted and oil-immiscible components of the reaction mixture, said oil-miscible reaction product being characterized by the presence of a group selected from the group consisting of



and



groups.

2. An improved Diesel fuel comprising a non-viscous petroleum oil and in admixture therewith a minor proportion, sufficient to decrease the ignition delay period of the fuel, of the oil-miscible product obtained by first reacting per-chloromethylmercaptan with a compound selected from the group consisting of compounds having the general formulae  $R(XH)_n$  and  $R(XM)_n$ , wherein R is selected from the group consisting of alkyl, aryl, alkaryl and aralkyl radicals, X is selected from the group consisting of oxygen and sulfur, M is a metal, and n is a whole number, and separating said oil-miscible reaction product from the unreacted and oil-immiscible components in the reaction mixture by water-washing and extracting with an organic solvent, said oil-miscible reaction product being characterized by the presence of a group selected from the group consisting of



and



groups.

3. An improved Diesel fuel comprising a hydrocarbon fuel oil and in admixture therewith a minor proportion of the oil-miscible product obtained by first reacting perchloromethylmercaptan with a phenol, and then separating said reaction product from the unreacted and the oil-immiscible components in the reaction mixture.

4. An improved Diesel fuel comprising a hydrocarbon fuel oil and in admixture therewith a minor proportion of the oil-miscible product obtained by first reacting perchloromethylmercaptan with a mercaptan other than perchloromethylmercaptan, and then separating said reaction product from the unreacted and oil-immiscible components in the reaction mixture.

5. An improved Diesel fuel comprising a hydrocarbon fuel oil and in admixture therewith a minor proportion of the oil-miscible product obtained by first reacting perchloromethylmercaptan with thiophenol, and then separating said

reaction product from the unreacted and oil-immiscible components of the reaction mixture.

6. An improved Diesel fuel comprising a non-viscous petroleum oil and in admixture therewith a minor proportion of the oil-miscible product obtained by first reacting perchloromethyl-mercaptan with a phenol and then separating said reaction product from the unreacted and oil-immiscible components of the reaction mixture, said reaction product being present in an amount sufficient to decrease the ignition delay period of the fuel.

7. An improved Diesel fuel comprising a non-viscous petroleum oil and in admixture therewith 15 a minor proportion of the oil-miscible product obtained by first reacting perchloromethylmercaptan with a mercaptan other than perchloromethylmercaptan and then separating said reaction product from the unreacted and oil-immiscible components of the reaction mixture, 20 said reaction product being present in an amount sufficient to decrease the ignition delay period of the fuel.

25 8. An improved Diesel fuel comprising a non-viscous petroleum oil and in admixture therewith a minor proportion of the oil-miscible product obtained by first reacting perchloromethyl-mercaptan with a thiophenol and then separating said reaction product from the unreacted and oil-immiscible components of the reaction mixture, said reaction product being present in an amount sufficient to decrease the ignition delay period of the fuel.

9. An improved Diesel fuel comprising a non-viscous petroleum oil and in admixture therewith a minor proportion of the oil-miscible product obtained by first reacting perchloromethyl-mercaptan with a compound selected from the group consisting of phenol, thiophenol, benzyl-mercaptan, ethyl alcohol, amyl mercaptan, and tertiary butyl mercaptan and then separating said reaction product from the oil-immiscible and unreacted components in the reaction mixture, said reaction product being present in an amount sufficient to decrease the ignition delay period of the fuel.

10. An improved Diesel fuel comprising a hydrocarbon fuel oil and in admixture therewith a minor proportion of the oil-miscible product obtained by first reacting perchloromethylmercaptan with a compound selected from the group consisting of phenol, thiophenol, benzyl mercaptan, ethyl alcohol, amyl mercaptan, and tertiary butyl mercaptan, and then separating said reaction product from the oil-immiscible and unreacted components in the reaction mixture.

60 11. An improved Diesel fuel comprising a hydrocarbon fuel oil and in admixture therewith a minor proportion, from about 0.1 per cent to about 5.0 per cent, of the oil-miscible product obtained by first reacting perchloromethylmercaptan with a compound selected from the group consisting of phenol, thiophenol, benzyl mercaptan, ethyl alcohol, amyl mercaptan, and tertiary butyl mercaptan, and then separating said reaction product from the unreacted and oil-immiscible components of said reaction mixture.

12. An improved Diesel fuel comprising a hydrocarbon fuel oil and in admixture therewith a minor proportion of the reaction product obtained by interreacting phenol with perchloro-methyl mercaptan in the presence of an alkaline hydroxide solution; extracting the reaction product from the reaction mixture with ether; and

distilling the ether extract to obtain said reaction product.

13. An improved Diesel fuel comprising a hydrocarbon fuel oil and in admixture therewith a minor proportion of the reaction product obtained by interreacting an ethyl alcohol solution of metallic sodium with perchloromethyl mer-

5 captan; water-washing the reaction mixture; extracting the reaction product therefrom with ether; and distilling the ether extract to obtain said reaction product.

EDWIN M. NYGAARD.  
JOHN H. McCACKEN.  
FRANCIS M. SEGER.